

March 15, 1949.

E. I. LARSEN ET AL  
METHOD OF BONDING A TUNGSTEN MEMBER  
TO A BACKING MEMBER  
Filed April 4, 1944

2,464,591

Fig. 1.



Fig. 2.



Fig. 3.



Fig. 4.



Fig. 5.



Fig. 6.



INVENTORS  
EARL I. LARSEN  
EARL F. SWAZY  
BY

Chester F. Carlson

ATTORNEY

## UNITED STATES PATENT OFFICE

2,464,591

## METHOD OF BONDING A TUNGSTEN MEMBER TO A BACKING MEMBER

Earl I. Larsen and Earl F. Swazy, Indianapolis, Ind., assignors to P. R. Mallory & Co., Inc., Indianapolis, Ind., a corporation of Delaware

Application April 4, 1944, Serial No. 529,533

3 Claims. (Cl. 113—112)

1

The present invention relates to composite articles and methods of making the same. More particularly the invention relates to the production of multi-metallic articles such as electrical contact elements, X-ray targets, spark gap electrodes, spark plug electrodes, welding electrodes, etc., in which one of the component members is formed of tungsten, and the other component is a material having physical properties different from those of tungsten.

It has been found that the chief cause of the failure or unsatisfactory performance of multi-metallic articles of the type mentioned above is due to distortion, warping or other surface changes thereof which sometimes produce cracks, fissures and the accelerated deterioration of these articles and which, in turn, are usually due to the difference in the coefficient of thermal expansion of the tungsten and the dissimilar material or materials.

Among the objects of this invention are: to avoid the above disadvantages and causes of failure; to provide a method of and means for producing composite metal articles free from incipient points of weakness and unrelieved stresses and strains which would cause accelerated deterioration of such articles; and to provide multi-metallic structures of increased strength and durability.

Other objects and advantages of this invention and details of manufacture and construction thereof will in part be obvious and will in part appear from the following description of preferred embodiments of the same when read in conjunction with the accompanying drawings, in which:

Figure 1 is a side view of the invention as applied to an X-ray target;

Figure 2 is a vertical section of an embodiment of the invention as applied to a contact or spark gap electrode;

Figures 3 through 6 are illustrative of a number of different embodiments of the invention.

The present invention relates especially to and has particular utility in the production of articles of the type mentioned above which may require relatively large and thin contact facing discs formed of tungsten. The invention contemplates overcoming the difficulties in the fabrication and operation of contact elements and X-ray targets of which tungsten is a constituent part of the contact facing by providing a special type of sintered backing composition for the tungsten contact facing; or, in some cases, by providing the special backing composition between the tung-

2

sten disc and the dissimilar material. In all cases the backing composition is characterized by a coefficient of thermal expansion close to that of tungsten, and at the same time, by the other physical properties required for the satisfactory service performance of the article in question, the composition being furthermore capable, when heated to a brazing temperature, of exuding a molten alloy adapted to wet and fuse with the tungsten facing and, where desired, with the dissimilar backing materials.

It has been found that backing compositions comprising the following ranges of ingredients satisfy the above requirements:

|    | A                                                               | B                                                                   |
|----|-----------------------------------------------------------------|---------------------------------------------------------------------|
|    | Compositions containing tungsten, nickel and copper             | Compositions containing tungsten, nickel and molybdenum             |
| 20 | Tungsten, 80 to 95%<br>Nickel, 10 to 2.5%<br>Copper, 10 to 2.5% | Tungsten, 60 to 95%<br>Nickel, 20 to 2.5%<br>Molybdenum, 20 to 2.5% |

It is within the scope of the invention to replace any desired proportion of either the copper or the molybdenum by the addition of gold. Furthermore, small percentages, i. e., up to about 1%, of manganese, cobalt, or iron may be incorporated in the sintered composition.

The following are typical examples of sintered backing compositions according to this invention:

|            | (I)        | (II)     |    |
|------------|------------|----------|----|
| 35         | Percent    | Percent  |    |
| Tungsten   | 90         | Tungsten | 90 |
| Molybdenum | 5          | Copper   | 4  |
| Nickel     | 5          | Nickel   | 6  |
|            | (III)      | (IV)     |    |
| 40         | Percent    | Percent  |    |
| Tungsten   | 90         | Tungsten | 85 |
| Copper     | 5          | Nickel   | 8  |
| Nickel     | 5          | Copper   | 8  |
|            | (V)        |          |    |
|            | Percent    |          |    |
| 45         | Tungsten   | 94       |    |
|            | Nickel     | 3        |    |
|            | Molybdenum | 3        |    |

In a typical method of carrying out this invention, suitable for example for making X-ray targets, a composition such as (I) above was ball-milled for 48 hours, impregnated with 1% of Glyptal resin as a binder, and screened through a 90 mesh sieve. The powder was then pressed to discs whose size would be correct after allowing for shrinkage during sintering. Since this

shrinkage may be as much as about 20%, the pressed discs were placed in a carbon boat on a thin layer of Alundum sand with a piece of Alundum slab between the sand and the bottom of the carbon boat, and sand was sprinkled over the Alundum to facilitate movement for the shrinkage during sintering. The carbon boat, with Alundum, sand, and the discs was placed into a sintering furnace and sufficient heat was applied to insure complete volatilization of the binder material, but not enough to exceed a black heat (about 500° C.). After the binder material had burned, the boat was gradually advanced into the heat, and after centering the discs in the hottest section, time was allowed for the boat to reach the sintering temperature which was about 1500° C. After a heating period of 20 minutes, the boat was pulled directly into the cooler. Tests and measurements indicated that the linear shrinkage during sintering was 15% to 19%, the hardness was 30 to 38 Rockwell C, and the density of the sintered discs was about 17.3 gms./cc.

Generally, the sintering temperature should be high enough to create a molten phase of the elements molybdenum-nickel (in the case of compositions (I) and (V) above), or copper-nickel (in the case of compositions (II), (III) and (IV) above), which results in a thorough diffusion of the two metals within each other with the formation of a eutectic alloy in certain instances. This molten alloy dissolves a portion of the powdered tungsten particles and exudes either the molybdenum-nickel or the copper-nickel phase, and it is this exuded molten phase which facilitates the subsequent brazing of the tungsten base composition to the tungsten discs, as described in more detail below.

After sintering as described, the discs were machined, and then brazed. According to this invention, advantage is derived from the lower melting point of the exuded nickel-molybdenum or nickel-copper alloy as well as from the phenomena involved in the fusion and freezing thereof, in order to effect the integral union of the alloy with the tungsten facing material. The liquid phase (nickel-molybdenum or copper-molybdenum) which exudes during the sintering is used as the chief constituent of the brazing medium. The brazing is effected by heating the tungsten disc in intimate contact with the tungsten base composition at a temperature adapted to insure sufficient fluidity of the liquid phase, which in Example I was about 1480° C. According to a preferred procedure, the tungsten base composition is placed upon and in direct contact with the upper surface of the tungsten disc; thus upon heating, the exuded molten phase of the backing member will be deposited by fusion upon and into the surface pores of the tungsten member, and during the freezing of the molten phase, any tungsten grains or particles which have entered into solution with the molten phase are precipitated out; thus resulting in a gradual duplex structure at the brazed joint in which there is a progressive enrichment of tungsten particles from top to bottom of the joint. Irrespective of the particular mechanism of fusion and solidification, micrographic examination of the brazed joint obtained by the process and materials of Example I showed that the molten phase of the tungsten base composition had diffused into the crystal structure of the tungsten disc and had formed a matrix cementing the two together.

Referring now to the drawings, Figure 1 shows a tungsten X-ray target 10 which, as shown, is embedded in the tungsten base composition 11, the latter being brazed, welded or otherwise secured to the supporting member 13 which may be made of copper.

Figure 2 shows a modification of the invention as applied to the fabrication of a contact or spark gap electrode, the tungsten facing disc 20 being integrally united with the tungsten base composition 21 along the brazed joint 22.

The embodiment of the invention illustrated in Figure 3 depicts a contact or spark gap electrode comprising a tungsten disc 30, and in which the backing member 31 of the tungsten base composition is brazed or welded to a further backing shape exemplified in the embodiment shown as a rivet 32 made of steel or any other desired metallic material.

The modification of the invention which is shown in Figure 4 represents a side view of a contact arm consisting of the tungsten contact facing disc 40 which is brazed directly to the backing material represented here as the contact arm 41.

Figure 5 is a sectional view through a welding electrode consisting of the tungsten facing disc 50, which is brazed to the tungsten base composition 51, the latter being screw-threaded into the body of the welding electrode 52. A water tube 53 is provided to cool the welding tip of the electrode member.

Figure 6 is a side view partly in section of a spark plug electrode, illustrating a further embodiment of the invention. The tungsten sparking member is represented at 60 and as shown, it is integrally united at 61 with the tungsten base composition 62 which in turn is united by screw threads 63 with the nickel rod 64.

It will be understood that discs, plates or other shapes, or facings of metallic tungsten could be secured to the backing member or members by a brazing or welding procedure different from the above embodiments, and that the invention is not limited to the use of the particular brazing procedure described, but that the invention is intended to be covered broadly within the spirit and scope of the appended claims.

What is claimed is:

1. The method of reducing distortion in a composite metal article of which one component member consists of tungsten in predominating proportions, which comprises contacting said member with a backing member of a composition containing about 60 to 95% tungsten, about 2.5 to 20% nickel and the remainder consisting of a third metal selected from at least one of the elements molybdenum and copper, and heating said members to a temperature sufficiently high as to create a molten phase of nickel and the third metal so that said molten phase exudes from said composition and unites said members by fusion.

2. The method of brazing a metallic material comprising a predominating proportion of tungsten to a metallic material having a coefficient of thermal expansion substantially different from that of tungsten, which comprises interposing between said two materials a composition containing about 60 to 95% tungsten, about 2.5 to 20% nickel and the remainder consisting of a third metal selected from at least one of the elements molybdenum and copper, and heating the composite article thus obtained to a temperature sufficiently high as to create a molten phase of

nickel and the third metal so that said molten phase exudes from said composition and fuses with said materials.

3. The method of brazing a tungsten facing metal to a backing member which comprises providing a backing member having a coefficient of thermal expansion close to that of said facing metal and composed of a ternary composition of tungsten, nickel and the remainder at least one of the elements molybdenum and copper, heating said member to a sintering temperature at which there exudes a binary liquid phase of said nickel and one of said third elements, heating the said facing metal in intimate contact with the said backing member to a temperature adapted to insure sufficient fluidity of said exuded binary phase whereby said exuded phase will be deposited by fusion upon and into the surface pores of the said facing metal and particles of said facing metal will enter into solution with said exuded phase, and cooling the combination

to securely bond the said facing metal to said backing member.

EARL I. LARSEN.

EARL F. SWAZY.

#### REFERENCES CITED

The following references are of record in the file of this patent:

#### UNITED STATES PATENTS

|    | Number    | Name        | Date           |
|----|-----------|-------------|----------------|
| 10 | 1,469,043 | Laise       | Sept. 25, 1923 |
|    | 1,625,427 | Rentschler  | Apr. 19, 1927  |
|    | 2,060,959 | Terry       | Nov. 17, 1936  |
| 15 | 2,096,924 | Schwatzkopf | Oct. 26, 1937  |
|    | 2,183,359 | Smithells   | Dec. 12, 1939  |
|    | 2,186,319 | Bilton      | Jan. 9, 1940   |
|    | 2,191,460 | Fisher      | Feb. 27, 1940  |
| 20 | 2,232,176 | Guthrie     | Feb. 18, 1941  |
|    | 2,234,834 | Scott       | Mar. 11, 1941  |
|    | 2,300,286 | Gwyn        | Oct. 27, 1942  |